

## UNITED STATES PATENT OFFICE

2,032,463

FIBERS DYED WITH WATER-INSOLUBLE  
AZO-DYESTUFFS

Alfred Bergdolt, Cologne-on-the-Rhine, Anton Ossenbeck, Cologne/Mulheim, and Ernst Tietze and Felix Gund, Cologne-on-the-Rhine, Germany, assignors to General Aniline Works, Inc., New York, N. Y., a corporation of Delaware

No Drawing. Application March 25, 1933, Serial No. 662,826. In Germany April 1, 1932

8 Claims. (Cl. 8—5)

The present invention relates to fibers dyed with water-insoluble azo-dyestuffs, more particularly it relates to fibers which are dyed with dyestuffs which may be represented by the probable general formula:



10

wherein  $x$  and  $y$  stand for radicals of the aromatic-, araliphatic- or aliphatic series, which are attached to the C-atoms of the carbonyl groups by carbon atoms, and which in case  $x$  and  $y$  stand for aliphatic radicals may be linked together,  $R$  stands for the radical of a diazotized diazotization component suitable for producing azo-dyestuffs, and wherein all nuclei may bear substituents which do not cause solubility in water;  $x$  and  $y$  may stand f. i., for methyl, ethyl, propyl, butyl, phenyl, naphthyl and benzyl. As substituents which may be present there are enumerated by way of example alkyl, alkoxy, halogen, and the nitro group, while the sulfonic acid group and the carboxylic acid group are excluded.

As coupling components coming into consideration for the purpose of our invention there may be mentioned for example acetylacetone, benzoylacetone, dibenzoylmethane, phenylacetylbenzoylmethane, the homologues and substitution products thereof.

As diazotization components there may be used all the bases free from groups inducing solubility in water generally used in the manufacture of azo-dyestuffs, for instance, amines of the benzene-, naphthalene- and carbazole series.

Our new dyeings are obtainable in the usual manner by diazotizing a primary amine and coupling on the fiber with a diketone of the kind referred to above; thereby generally yellowish to orange shades of good fastness properties are obtained, the dyeings being dischargeable, yielding clear white discharges.

The invention is illustrated by the following examples, without being limited thereto:

Example 1.—15 grams of dibenzoylmethane are intimately mixed with 60 ccs. of alcohol, 30 ccs. of water and 7.5 ccs. of aqueous caustic soda lye of 38° Bé. strength and stirred into 900 ccs. of water containing 5 ccs. of aqueous caustic soda lye of 38° Bé. strength and 10 ccs. of aqueous Turkey red oil of 50% strength.

55 Cotton yarn is impregnated in this solution for

about half an hour, squeezed, dried, and the dyeing is developed by passing the yarn for half an hour into a diazo solution prepared from 22.5 grams of 1-methyl-2-amino-4-chloro-5-benzoylaminobenzene, said diazo solution containing 11 ccs. of aqueous acetic acid of 50% strength.

The cotton is rinsed, washed, soaped in a boiling bath, washed again and dried. A clear greenish-yellow dyeing of good fastness to boiling and light is thus obtained, said dyeing being 10 dischargeable, yielding thereby clear white discharges. The dyestuff corresponds to the following formula:



15



20



25

Example 2.—15 grams of benzoyl-p-chlorobenzoylmethane are dissolved as described in Example 1. Cotton yarn is impregnated with this solution for about half an hour, rinsed, dried, and the dyeing is developed in a diazo solution prepared from 21 grams of 1-chloro-2-amino-4-methoxy-5-benzoylaminobenzene. After washing, soaping in a boiling bath, washing again and drying, a clear reddish yellow of good fastness to boiling and light is obtained. The dyeing can be discharged.

The dyestuff corresponds to the following formula:



40



45



50

Example 3.—In an analogous manner as described in Example 1, the dyestuff produced from p-tolylbenzoylmethane and diazotized 2,4'-dimethyl-5-methoxy-2'-nitro-4-aminoazobenzene 55

on cotton yields an orange fast to boiling and light. The dyeing is dischargeable.

The dyestuff corresponds to the following formula:



In the following table there are given some 20 combinations and the shades obtained thereby when prepared on celulosic fibres according to the directions given in Example 1:

|    | Coupling component            | Diazotization component                             | Shade            |
|----|-------------------------------|-----------------------------------------------------|------------------|
| 25 | Acetylacetone                 | 1,4-diethoxy-2-amino-5-benzoylaminobenzene.         | Orange.          |
|    | Benzoylacetone                | 3-nitro-1-aminobenzene.                             | Yellow.          |
|    | Diketohydridene               | <i>a</i> -aminoanthraquinone.                       | Orange.          |
| 30 | Dibenzoylmethane              | 1-amino-2-chloro-4-benzoyl-5-methoxybenzene.        | Reddish yellow.  |
|    | Do                            | 2,4'-dimethyl-5-methoxy-2'-nitro-4-aminoazobenzene. | Orange.          |
|    |                               | 1-amino-2-chloro-4-benzoyl-5-methylbenzene.         | Reddish yellow.  |
|    |                               | 1-amino-2-methyl-4-benzoyl-5-methoxybenzene.        | Golden orange.   |
| 35 | Do                            | 1-amino-2-chloro-4-benzoyl-5-methoxybenzene.        | Golden yellow.   |
|    | Do                            | 1-amino-2-methoxy-4-benzoylaminobenzene.            | Orange.          |
|    | Do                            | 1-amino-2,5-dimethoxy-4-benzoylaminobenzene.        | Orange.          |
|    | Do                            | 1-amino-2,5-dimethoxy-4-benzoylaminobenzene.        | Orange.          |
| 40 | Do                            | 1-amino-2-ethoxy-4-benzoyl-5-methylbenzene.         | Golden yellow.   |
|    | Do                            | 1-amino-2-methoxy-4-benzoylaminobenzene.            | Golden yellow.   |
|    | Do                            | 1-amino-2-chloro-4-benzoylaminobenzene.             | Reddish yellow.  |
|    | Do                            | 1-amino-2-chloro-4-methyl-5-benzoylaminobenzene.    | Reddish yellow.  |
| 45 | Do                            | 1-amino-2-methyl-4-chloro-5-benzoylaminobenzene.    | Greenish yellow. |
|    | Do                            | 1-amino-2-chloro-4-methoxy-5-benzoylaminobenzene.   | Reddish yellow.  |
|    | Do                            | 1-amino-2-methoxy-4-chloro-5-benzoylaminobenzene.   | Greenish yellow. |
| 50 | 2-methylbenzoylbenzoylmethane | 1-amino-2-methyl-4-benzoyl-5-chlorobenzene.         | Reddish yellow.  |
|    | 4-chlorobenzoylbenzoylmethane | 2,5-dichloroaniline.                                | Yellow.          |
|    | Do                            | 1,3-dimethyl-4-amino-6-benzoylaminobenzene.         | Greenish yellow. |
|    | Do                            | 2,3'-dimethyl-4-amino-azobenzene.                   | Yellowish brown. |
| 55 | We claim:                     |                                                     |                  |

1. Cellulosic fibers dyed with a water-insoluble azo-dyestuff of the following general formula:



65 wherein  $x$  and  $y$  stand for radicals of the aromatic-, aromatic-aliphatic- or aliphatic series, R stands for the radical of a diazotized substituted amine of the aromatic series, and wherein in the nuclei bear only substituents which do not cause solubility in water and which are selected from the group consisting of alkyl, alkoxy, halogen, nitro and acylamino, the shades produced being generally yellow to orange and being dischargeable to a pure white.

2. Cellulosic fibers dyed with a water-insoluble azo-dyestuff of the following general formula:



10 wherein  $x$  and  $y$  stand for radicals of the aromatic-, aromatic-aliphatic- or aliphatic series, R stands for a substituted radical of the benzene- or naphthalene series, and wherein the nuclei bear only substituents which do not cause solubility in water and which are selected from the group consisting of alkyl, alkoxy, halogen, nitro and acylamino, the shades produced being generally yellow to orange and being dischargeable to a pure white.

3. Cellulosic fibers dyed with a water-insoluble azo-dyestuff of the following general formula:



30 wherein  $x$  and  $y$  stand for radicals of the phenyl series, R stands for the radical of a diazotized substituted amine of the aromatic series, and wherein the nuclei bear only substituents which do not cause solubility in water and which are selected from the group consisting of alkyl, alkoxy, halogen, nitro and acylamino, the shades produced being generally yellow to orange and being dischargeable to a pure white.

4. Cellulosic fibers dyed with a water-insoluble azo-dyestuff of the following general formula:



50 wherein  $x$  and  $y$  stand for radicals of the phenyl series, R stands for a substituted radical of the benzene- or naphthalene series, and wherein the nuclei bear only substituents which do not cause solubility in water and which are selected from the group consisting of alkyl, alkoxy, halogen, nitro and acylamino, the shades produced being generally yellow to orange and being dischargeable to a pure white.

55 5. Cellulosic fibers dyed with a water-insoluble azo-dyestuff of the following formula:



70 yielding clear greenish-yellow, dischargeable dyes of good fastness to boiling and light.

6. Cellulosic fibers dyed with a water-insoluble azo-dyestuff of the following formula:



15 yielding clear reddish yellow dyeings of good fastness to boiling and light.

7. Cellulosic fibers dyed with a water-insoluble azo-dyestuff of the following general formula:



25 wherein  $x$  and  $y$  stand for methyl groups, R stands for the radical of a diazotized substituted

amine of the aromatic series, and wherein the nuclei may bear substituents selected from the group consisting of alkyl, alkoxy, halogen, nitro and acylamino, the shades produced being generally yellow to orange and being dischargeable to a pure white. 5

8. Cellulosic fibers dyed with a water-insoluble azo-dyestuff of the following general formula:



wherein  $x$  and  $y$  stand for methyl groups, R stands for a substituted radical of the benzene- or naphthalene series, and wherein the nuclei may bear substituents selected from the group consisting of alkyl, alkoxy, halogen, nitro and acylamino, the shades produced being generally yellow to orange and being dischargeable to a pure white. 15 20

ALFRED BERGDOLT.

ANTON OSSENBECK.

ERNST TIETZE.

FELIX GUND.

25